

# UNITED STATES PATENT OFFICE.

JOHN F. JAMES, OF HOUSTON, TEXAS.

## FURNITURE-POLISH.

1,363,419.

Specification of Letters Patent. Patented Dec. 28, 1920.

No Drawing.

Application filed November 7, 1919. Serial No. 336,328.

To all whom it may concern:

Be it known that I, JOHN F. JAMES, a citizen of the United States, residing at Houston, Harris county, Texas, have invented a certain new and useful Improvement in Furniture-Polish, of which the following is a full, clear, and exact description, such as will enable others skilled in the art to which it appertains to make and use the same.

10 My invention relates to an improvement in polishing compounds for use in cleaning and polishing furniture, vehicles, woodwork and other similarly coated or enameled surfaces.

15 The object of my invention is to provide a liquid compound of the character described which will be economical to manufacture and which will serve to clean tarnished surfaces and restore their original luster and finish and which will quickly dry, leaving a clean smooth surface. I have found by experiment that it is desirable in a good furniture or vehicle polish to combine a cleansing agent, a renewing agent and a 25 drying agent. The cleansing agent must be such as will remove grease or stain from the polished surface but which will not injure the finish thereof or counteract the beneficial effects of the other ingredients. The

30 renewing agent should have the qualities of a wax or light varnish without any viscous or sticky quality, while the drying agent should be such as to cause the surface to dry almost immediately after application.

35 The larger portion—about  $\frac{2}{3}$  of the compound—is necessarily a light grade of light mineral or vegetable oil, preferably a petroleum distillate of paraffin base. Some good grade of castor oil might serve as an equivalent of my preferred oil, but this oil is entirely too expensive and is at best simply a substitute for the preferred ingredient.

40 I mix with the oil about half as much good cleansing agent adapted to remove grease and brighten the tarnished surface. 45 I prefer to use for such agent a good quality of acid vinegar. This has been found to be most efficient. Ammonia will also act in the same capacity, but not with the same efficiency.

I then supply a small quantity—about 0.1 of the volume of oil—of turpentine. This acts with the oil to smooth and reename the surface, and also assists in drying the mixture. To this compound I then add a small 55 quantity of camphor to act as a further drying agent. I find that the quantities by weight of the separate ingredients necessary to produce the greatest efficiency are as follows:

|                    |         |
|--------------------|---------|
| Light paraffin oil | 62.5%   |
| Acid vinegar       | 31 %    |
| Turpentine         | 6 %     |
| Camphor            | 0.5% 65 |

The exact proportions of these ingredients might be varied slightly, but in the proportions above stated the most efficient compound is produced. The separate ingredients when properly mixed do not easily 70 separate and serve to form a composition easily applied and very effective in both cleansing and polishing. It dries quickly and will gather no dust, thus leaving a clean luster closely like the original finish. It 75 may be applied with a soft cloth or sponge and need only be rubbed smooth with a dry cloth or chamois and the finish will be restored.

Having thus described my invention, what 80 I claim as new and desire to protect by Letters Patent is:

1. A furniture polish composed of 62.5% light paraffin oil, 31% of acid vinegar, 6% turpentine, and about  $\frac{1}{2}$  of 1% of camphor. 85

2. A furniture polish composed of 62.5% of a light grade of oil, 31% of acid vinegar, 6% of turpentine and  $\frac{1}{2}$  of 1% of camphor.

3. A furniture polish composed of about 90  $\frac{2}{3}$  by weight of light paraffin oil, of slightly less than  $\frac{1}{3}$  by weight of acid vinegar, about  $\frac{1}{10}$  by weight of turpentine and a fraction of 1% of a drying agent.

In testimony whereof, I hereunto affix my 95 signature this the 3rd day of November, A. D. 1919.

JOHN F. JAMES.